

## UNITED STATES PATENT OFFICE.

JACOB SHOTWELL ROBESON, OF PENNINGTON, NEW JERSEY.

## FUEL BRIQUETTE AND METHOD OF MAKING SAME.

No Drawing.

Application filed September 26, 1924. Serial No. 740,040.

In the manufacture of fuel briquettes from coal dust or coal in other finely subdivided form, it is common practice to add a binding agent, press the mixture into the desired form and bake or otherwise heat the briquettes to dry or harden them. Most binding agents used for this purpose are of lower fuel value than the coal so that the average B. t. u. of the mixture is reduced and the heating tends to further reduce the B. t. u. by the driving off of volatile combustible constituents of the coal.

Various attempts have been made to render fine coal better adapted for use as fuel and to increase the B. t. u. thereof by adding oil, but such oil and coal dust mixture is difficult to handle, and in most cases results in a very smoky flame. So far as I know, attempts to form briquettes from a coal dust and oil mixture have not been satisfactory.

My present invention involves a new method of forming briquettes from coal dust and oil mixtures, and also involves a new briquette as an article of manufacture.

My new briquette has very high fuel value, due to the fact that it retains a comparatively large percentage of the oil and other volatile parts of the fuel mixture; it may be burned with comparatively little or no smoke; it has a hard outer wall or casing rendering it adapted for storage, shipment or rough handling; the cost of manufacture is comparatively low, due to the low temperature employed in the baking or hardening step of the process; and the product is commercially very satisfactory.

In my improved process I add to the oil and coal dust mixture a solid water-soluble quick hardening adhesive or binder which will unite with the small percentage of water normally present in the oil and coal dust mixture, and will serve to give to the briquette the desired strength while the briquette is "green", that is, after it is pressed to the desired form or otherwise shaped, and before it is baked or hardened. During the baking or hardening process the temperature is kept comparatively low, that is, between 150° and 250° C., which acts to set the binder or adhesive which was added, to drive off the moisture, and to drive out the volatile combustible constituents of the surface portions of the briquette. The heating does not drive out any considerable portion of the volatile combustible constituents

from the interior of the briquette, but it serves to coke the outer surface parts so as to form a hard shell.

The percentage of volatile matter in the briquette increases as the distance from the outer surface increases, but the interior portion containing the highest percentage of volatile matter is protected by the outer shell not only during shipment and storage, but also when the briquette is thrown onto the fire. The oil and other volatile constituents are not driven off until after the outer surface of the briquette begins to burn at a good white heat, and then are driven off comparatively slowly so that they are burned to yield their full heating value without producing a smoky flame. The percentage of ash in the briquette is lower than with the ordinary briquette, due to the presence of the oil constituent.

I do not wish to be limited to any exact proportion of coal dust and oil, but have secured satisfactory results with the oil running as high as 20 per cent. Either anthracite or bituminous coal may be employed, and the coal dust may be used in the usual form or may be ground or crushed to a very much finer form, and in being mixed with the oil may produce a mixture analogous to or actually constituting an amalgam. What is known as "Trent amalgam" may be used very satisfactorily. This includes about 80% to 82% very fine coal, 14% to 16% oil, and 2% to 4% moisture.

As a binding agent to give to the mixture its green strength, I preferably employ about 2% of lignone powder resulting from the evaporation of sulfite cellulose liquor to dryness. Such a powder acts to absorb the small percentage of moisture present in the oil-coal mixture and thereby forms the adhesive to hold the mixture together, particularly when green. Instead of using this sulfite cellulose liquor powder or lignone, I may employ other dry quick-setting water-soluble adhesive, such as flour, dextrine or the like. I may employ other adhesives or binders including moisture or water, but obviously it is desirable to add as little water or other non-combustible matter as possible. In forming the mixture into briquettes I preferably employ a properly designed extrusion machine to force the mixture through a die or aperture in the form of a solid or tubular rod or bar which may be cut or broken into sections or shapes of the desired length.

The forcing is preferably done by an auger so as to get continuous delivery, although a plunger might be employed. The heating should be continued only sufficiently long 5 to harden or coke the outer surface of the briquette without driving out the volatile constituents from the interior. The more of the combustible volatiles that are left in, the greater will be the fuel value of the briquette, but the heating should be carried sufficiently far to properly carbonize or harden the outer shell or surface portion. The shorter the heating period the lower the manufacturing cost. The heat drives off all 10 of the water and most of the lighter oils, but these latter may be condensed and collected as it is of course understood that the heating is conducted out of contact with the air.

By using 2% of lignone with Trent amalgam, the anthracite coal of which contained 20 4% to 7% volatiles, shaping with an auger machine and baking at 200° C. until sufficiently hard to stand transportation, I have produced very satisfactory briquettes containing 10% to 15% of combustible volatile constituents.

I have discovered that coal or other mineral matter having too high a fluid content of such a liquid as oil, bitumen, asphalt or 30 other non-water-soluble adhesive, can be mixed with lignone, liquid or dry, or other quick-setting water-soluble adhesive, and formed into suitable briquettes in an extrusion machine, by forcing through a die by the use of a screw or auger.

In the foregoing description I have used the term "coal dust" to include any form of coal or other combustible mineral matter in finely subdivided form. The coal particles may all pass a 200 mesh sieve, or the coal 40 may be or include "buckwheat" coal, 10% to 30% of which will remain on a 10 mesh sieve. In order to secure proper working in the extrusion machine it is important that the mixture be plastic, and the plasticity is greater when the finer grades of coal dust are used. Also by using the finer grades of coal dust, the briquette is made more dense and with smaller interstitial spaces between the 50 coal particles and less of the volatile constituents escape from the interior of the briquette during the heating operation.

I have used the term "oil" to include not only what is commonly known as "oil", but 55 also bitumen, asphalt or other combustible liquid of the same general type, and whether used in the crude form or obtained in the distillation or purification of mineral oil, or distillation from coal, lignite or the like. 60 The oil serves as a non-water soluble binder to hold the dust together as the non-volatilized portions aid in uniting the particles during the heating.

Although the briquettes may be of solid 65 form they are preferably made of tubular

form so as to give increased burning surface and free passages for the access of air thereto during the burning.

Having thus described my invention, what I claim as new and desire to secure by Letters Patent is:

1. A fuel briquette of tubular form, including fine coal, oil and lignone, the surface portions being harder than the inner portions, and containing a lower percentage 75 of volatile matter.

2. A method of forming briquettes which includes mixing a mineral fuel in granular or powdered form with a non-water-soluble adhesive binder, adding a water-soluble adhesive, pressing the same into suitable shapes, and heating the shaped masses to drive off the volatiles from the exposed surfaces of such masses.

3. A method of making briquettes which includes mixing fine coal with a liquid fuel, adding a water-soluble adhesive, forming into suitable masses by exerting pressure thereon, and heating to distill off a portion only of the liquid and to coke the surface 90 portion.

4. A method of making briquettes which includes mixing coal dust with oil, adding a solid adhesive, forming into suitable masses by exerting pressure thereon, and heating the formed masses to a temperature below 250° C.

5. A method of forming briquettes which includes adding lignone to a mixture of coal dust and oil, forming the mixture into suitable shapes and heating.

6. A method of forming briquettes which includes adding lignone to a mixture of fine coal and oil, forming the mixture into suitable shapes and heating at a low temperature 105 to drive off a portion only of the volatile constituents.

7. A method of manufacturing briquettes which includes adding lignone powder to a mixture of fine coal and oil, forming masses of the mixture, and heating said masses to a temperature not above 250° C.

8. A method of forming briquettes which includes adding a small percentage of dry lignone to a mixture of coal dust and 15% to 20% of oil, forming into suitable masses upon an extrusion machine, and heating to distill off a portion only of the oil.

9. A method of forming briquettes which includes adding a small percentage of dry adhesive in powder form to a mixture of coal dust and from 15% to 20% of oil, forming into suitable masses upon an extrusion machine, and heating such masses to coke the outer surface portion thereof but not to distill all of the oil from the inner portions.

10. A method of forming briquettes which includes mixing coal dust with 15% to 20% of a mineral oil, and approximately 2% of dry lignone, forming the mixture into suit- 130

able shapes, and heating the shapes at a temperature between 150° and 200° C. to drive off the volatile constituents from the exposed surface portions and effect coking 5 at such surfaces.

11. The method of making fuel briquettes which includes forcing a plastic mass of finely subdivided solid fuel and a binder through an aperture to form a rod, subdividing the rod into sections to drive off volatile matter from the surface portions, and heating the sections to harden the same. 10

12. The method of making fuel briquettes which includes forming a plastic mass of finely subdivided solid fuel, substantially 15 all of which will pass a 200 mesh screen and a binder, forcing said mass through an aperture to form a rod, subdividing the rod into sections, and heating the sections to drive 20 off volatile matter from the surface portions to harden the same.

13. The method of making fuel briquettes, which includes mixing coal dust and a binder, forcing the mixture through an aperture to form a continuously delivered rod, causing said rod to break up into sections, 25 and heating said sections to drive off volatile matter from the surface portions to harden the same.

14. The method of forming briquettes 30 which consists in adding a solid water-soluble binder to a mixture of oil and finely subdivided solid fuel, forcing the same through an aperture to form a continuously delivered rod, breaking the rod into comparatively 35 short sections to drive off volatile matter from the surface portions, and heating the sections to harden the exterior thereof.

15. A briquette made by adding a solid 40 water-soluble binder to a mixture of oil and finely subdivided solid fuel, forcing the same through an aperture to form a continuously delivered rod, breaking the rod into comparatively short sections to drive 45 off volatile matter from the surface portions, and heating the sections to harden the exterior thereof.

16. A briquette in the form of a section of a rod having a substantially smooth peripheral surface and broken end surfaces, 50 the briquette including a solid finely subdivided fuel and a binder, and hardened by heating to drive off volatile matter from the surface portion after forming.

Signed at Pennington in the county of 55 Mercer and State of New Jersey this 13 day of September A. D. 1924.

JACOB SHOTWELL ROBESON.